

June 12, 1934.

W. CASE

1,962,682

LAMINATED MATERIAL

Filed June 22, 1932

FIG. 1.



FIG. 2.



FIG. 3.



FIG. 4.



William Case,  
Inventor,  
Delos G. Haynes,  
Attorney.

## UNITED STATES PATENT OFFICE

1,962,682

## LAMINATED MATERIAL

William Case, St. Louis, Mo., assignor to Bemis  
Bro. Bag Co., St. Louis, Mo., a corporation of  
Missouri

Application June 22, 1932, Serial No. 618,632

6 Claims. (Cl. 154—50)

This invention relates to laminated materials, and with regard to certain more specific features, to laminated materials comprising, generally, fabric layers secured to paper layers, adapted for use in the manufacture of lined bags.

Among the several objects of the invention may be noted the provision of laminated fabrics of the class described in which asphalt is used as an adhesive to join together two or more of the layers, but in which the fabric layer is so treated as to be resistant to stains caused, for example, by softening of the asphalt with excessive heat, pressure, solvent action, or the like; the provision of a fabric of the class described which has improved waterproof, as well as acid- and alkali-proof, qualities; and the provision of a fabric of the class described wherein the fabric layer, for example, burlap, is treated so that its tendency to "shed" fibers and the like is eliminated or greatly minimized. Other objects will be in part obvious and in part pointed out hereinafter.

The invention accordingly comprises the elements and combinations of elements, features of construction, and arrangements of parts which will be exemplified in the structures hereinafter described, and the scope of the application of which will be indicated in the following claims.

In the accompanying drawing, in which are illustrated several of various possible embodiments of the invention:

Fig. 1 is an enlarged section showing one embodiment of the invention;

Fig. 2 is an enlarged section showing a second embodiment of the invention;

Fig. 3 is an enlarged section showing a third embodiment of the invention; and,

Fig. 4 is an enlarged section showing a fourth embodiment of the invention.

Similar reference characters indicate corresponding parts throughout the several views of the drawing.

Lined fabric is a commodity well-known in the bag manufacturing art. Bags made from such lined fabric are used chiefly for deliquescent and like materials.

Heretofore the customary construction of such lined or laminated fabrics has been substantially a layer of fabric (usually burlap), having affixed thereto with asphalt a layer of paper (usually crepe paper). Frequently a further layer of paper is affixed, also with asphalt, to the first paper layer. A fault of this material is that when hot materials are charged into bags constructed therefrom, the asphalt softens and the fabric is badly stained thereby. Such staining

renders the bags prematurely old-appearing, and further makes them difficult to handle, as the stained fabric is tacky and adjacent bags tend to stick together to an undesirable extent.

Asphalt cannot economically be done away with entirely, and substituted by other adhesives to cure this staining problem, because in the first place, no other adhesive can compete with asphalt as regards its cost, and in the second place, it has many desirable qualities (flexibility, sufficient tackiness, water-imperviousness, acid and alkali resistance, and the like) which substitute adhesives do not offer. For this reason, the cure for the staining problem is more advantageous if it does not require the elimination of asphalt entirely from the material.

The present invention falls within the last category. Briefly, the present invention comprises protecting the fabric layer with a coating of rubber material, whereby it is rendered impervious (and hence unstainable) by the heated asphalt adhesive.

Referring now more particularly to Fig. 1, there is illustrated at numeral 1 a fabric layer, such as burlap. Secured to the burlap 1 by a layer of coagulated latex 2 is a layer of crepe or like lining paper 3. A layer 4 of asphalt (relatively thicker than the rubber-latex layer 2) binds a second paper layer 5 to the paper layer 3.

The paper layers 3 and 5 are usually impervious to the asphalt layer 4, even when it is warmed or softened. But even if the layer 3 is somewhat pervious, the latex layer 2 so protects the burlap 1 that no asphalt can penetrate therethrough and stain the burlap 1. The asphalt layer 4, however, provides the principal water-proofing medium, as in prior materials.

In Fig. 2 is illustrated another embodiment of the invention in which a latex or rubber layer 6 is affixed to one side of the burlap 1, while the asphalt layer 4 joins the other side of the burlap 1 to the paper liner 3. In this embodiment, the latex 6 sufficiently penetrates the burlap to render it impervious to the asphalt 4, even though the asphalt 4 directly adjoins the burlap. This is because the burlap is practically impregnated with the latex, and the latex is repellent to the staining, warmed asphalt.

The Fig. 3 embodiment of the invention is quite similar to the Fig. 2 embodiment, the only change being that a further layer 7 of asphalt and a layer 8 of paper are affixed to the first paper layer 3. This embodiment is particularly suited for extreme conditions, such as the storage of calcium chloride and the like.

In the Fig. 4 embodiment of the invention, layers of latex 6 and 2 are applied to both outer and inner sides of the fabric 1, respectively, thus securing an additional protective effect. The Fig. 4 embodiment is otherwise similar to the embodiments shown in the other figures.

From the foregoing descriptions, it will be seen that the rubber latex layer exerts a protective effect on the fabric regardless of the side upon which it is positioned. In Fig. 1, the latex is between the asphalt and the burlap, while in Figs. 2 and 3 it is on the opposite side of the burlap from the asphalt. It is efficacious to prevent staining in either position.

While latex adhesives are considered to be the most desirable rubber material for the purposes of the present invention, other rubber materials may be used. For example, benzol solutions of rubber, gutta-percha, balata, or the like may be used to form the layers by allowing the benzol to evaporate. When the latex is properly coagulated, particularly in the Fig. 2 and Fig. 3 embodiments, it is not tacky and the bags may be piled one on top of the other without sticking together.

A distinctly important advantage accrues to the Fig. 2, Fig. 3 and Fig. 4 embodiments, in that the outer latex layer 6 effectively prevents the burlap 1 from shedding fibers or lint as it is handled. This is particularly advantageous when the material is formed into bags and used for packaging foodstuffs, such as granulated sugar, in which event the foodstuff is not contaminated with burlap fibers or lint.

It will be understood that, although the accompanying drawing shows asphalt and rubber layers of considerable thickness, this is done for clarity only, and in practice the layers are relatively quite thin. The rubber, as has been indicated, is desirably in the form of latex or latex compounds when applied, and the layers 2 and 6 may be so thin as not to be altogether continuous (although continuity is desirable). Layer 2 is sufficiently continuous, however, to prevent the asphalt from migrating into the fabric or through the openings in the weave to the face of the fabric. Layer 6 is preferably a wash coating penetrating the fibers of the fabric to some extent, and partially encircling them, and to some extent forming films in the openings of the weave of the fabric.

In view of the above, it will be seen that the

several objects of the invention are achieved and other advantageous results attained.

As many changes could be made in carrying out the above constructions without departing from the scope of the invention, it is intended that all matter contained in the above description or shown in the accompanying drawing shall be interpreted as illustrative and not in a limiting sense.

I claim:

1. A laminated material particularly adapted for manufacture into bags comprising a layer of fabric, at least one layer of paper, and at least one layer of asphalt adhesive, and a layer of rubber positioned with respect to said fabric so as to prevent the same from being substantially stained by said asphalt.

2. In a laminated material comprising layers of fabric and paper and adhesive asphalt, means for preventing said asphalt from substantially staining said fabric comprising a layer of rubber.

3. A laminated material comprising a layer of fabric, a layer of rubber derived from latex on one side of said fabric and penetrating the same, a layer of asphalt on the other side of said fabric, and a layer of paper joined to said fabric by the said asphalt layer.

4. A laminated material comprising a layer of fabric, a layer of rubber derived from latex on one side of said fabric and penetrating the same, a layer of adhesive material on the other side of said fabric, and a layer of paper joined to said fabric by the said layer of adhesive material.

5. A laminated material comprising a layer of fabric, a layer of rubber derived from latex juxtaposed to said fabric layer, a layer of paper juxtaposed and joined to said rubber layer, a layer of adhesive material juxtaposed and joined to said paper layer, and a second layer of paper juxtaposed and joined to the other side of said adhesive layer.

6. A laminated material comprising a layer of fabric, layers of rubber derived from latex juxtaposed to said fabric layer on both sides thereof and penetrating the same, a layer of paper juxtaposed and joined to one of said rubber layers, a layer of adhesive material juxtaposed and joined to said paper layer, and a second layer of paper juxtaposed and joined to the other side of said adhesive layer.

WILLIAM CASE.

130

135

140

145

150